

## UNITED STATES PATENT OFFICE

2,298,280

## TREATMENT OF METAL

Wilfred James Clifford and Henry Heward Adams,  
Brentford, England, assignors to Parker Rust-  
Proof Company, Detroit, Mich., a corporation  
of Michigan

No Drawing. Original application February 2,  
1939, Serial No. 254,238. Divided and this ap-  
plication March 21, 1941, Serial No. 384,541. In  
Great Britain February 4, 1938

5 Claims. (Cl. 148—6.5)

This invention relates to the treatment of metals, especially iron or steel, for instance to the treatment of metals with phosphate coating solutions in order to improve the resistance of the metals to corrosion or to provide a corrosion-resisting base for paints.

It is an object of the invention to accelerate the action of reagents which attack a metal surface.

It is a further object of the invention to accelerate the action of phosphate coating solutions, i. e., to reduce the time taken by the coating solution to form a complete coating, or to reduce the temperature, or to obtain a better coating in a given time under given conditions than if the compounds were not present.

Where phosphate and similar coating solutions are being employed, they may be applied to the metal in any suitable manner, for instance by spraying, brushing, flowing or immersion methods.

We have found that the action of reagents which attack metal surfaces, and especially phosphate coating solutions, can be accelerated by incorporating hydroxylamine therein.

The cleaned steel sheet in the examples given below is a steel sheet in its original bright rolled condition rendered substantially free from grease by wiping with clean white spirit.

While the hydroxylamine may be the only accelerator present in a coating bath, it may also be employed in conjunction with other accelerators, for instance metallic accelerators such as copper compounds or oxidizing agents such as nitrates or nitrites. The presence of copper ions appears to promote heavier and darker coatings, and the presence of a nitrate such as zinc nitrate appears to give a slight further acceleration.

The optimum concentration of the accelerating compound in the reagent attacking the metal surfaces differs with different compounds but in the case of phosphate coating solutions is in general from about .01% to .4% by weight of the solution. Too much or too little of the accelerating compound may be detrimental to good results. 45

The invention is illustrated by the following examples:

## Example 1

A cleaned steel sheet can be successfully coated by treating it with an N/5 solution of zinc dihydrogen phosphate (determined by phenol-phthalein) containing 0.4% of hydroxylamine, at a temperature of 80° C.

## Example 2

A cleaned steel sheet can be successfully coated by treating it at a temperature of 15° to 80° C. with an N/5 solution of manganese dihydrogen phosphate (determined by phenol-phthalein) containing 0.4% of hydroxylamine.

If in any of the above examples 0.001% of copper (calculated as the metal) is added to the solution, for instance in the form of the nitrate or carbonate, a darker and slightly heavier coating is obtained, and the addition of zinc nitrate results in a slightly further acceleration.

20 What we claim is:

1. A coating solution containing a coating acid phosphate and hydroxylamine in an amount that accelerates the coating action of the solution.

2. A coating solution containing zinc coating acid phosphate and hydroxylamine in an amount that accelerates the coating action of the solution.

3. The process which comprises treating ferrous surfaces with a phosphate coating solution, the action of which is accelerated by hydroxylamine until a corrosion-resistant paint-holding coating is obtained.

4. A process which comprises treating ferrous surfaces with a zinc phosphate coating solution accelerated by hydroxylamine until a corrosion-resistant paint-holding coating is obtained.

5. The process which comprises dissolving in a solution materials comprising hydroxylamine and the ingredients of a coating acid phosphate in amounts resulting in an accelerated phosphate coating bath, and treating a ferrous surface with the solution until a phosphate coating is formed upon said surface.

WILFRED JAMES CLIFFORD.  
HENRY HEWARD ADAMS.